# EUROPEAN PATENT SPECIFICATION

(11) **EP 1 498 506 B1**
(45) Date of publication and mention of the grant of the patent: **28.06.2006**
(21) Application number: 04023082.3
(22) Date of filing: 14.02.2001
(51) Int. Cl.: C22C 38/00, C22C 38/06, C22C 38/58, C21D 9/46, C22C 38/04, C21D 8/02

(54) **High tensile strength cold-rolled steel sheet having a high r-value, excellent strain age hardenability and natural aging resistance and method of producing the same**
Hochfestes Kaltgewalztes Stahlblech mit hoch r-Wert, exzellenter Reckalterungseigenschaften und Alterungsbeständigkeit sowie Verfahren zur dessen Herstellung
Tôle d'acier à haute resistance laminée a froid ayant une haute r-valeur, excellente aptitude au durcissement au vieillissement par écrouissage et son procédé de fabrication

(30) Priority: 26.05.2000 JP 2000156274; 28.06.2000 JP 2000193717; 27.10.2000 JP 2000328924; 02.11.2000 JP 2000335803
(43) Date of publication of application: 19.01.2005
(62) Divisional of application: 01906128.2
(73) Proprietor: JFE Steel Corporation, Tokyo (JP)
(72) Inventor: Kami, Chikara, Technical Research Laboratories, Chiba-shi Chiba, 260-0835 (JP); Tosaka, Akio, c/o Chiba Works, Chiba-shi Chiba, 260-0835 (JP); Yamazaki, Takuya, Technical Research Laboratories, Chiba-shi Chiba, 260-0835 (JP)
(74) Representative: Grünecker, Kinkeldey, Stockmair & Schwanhäusser Anwaltssozietät

(56) References cited:
- EP-A- 0 608 430
- EP-A- 0 943 696
- US-A- 4 838 955
- US-A- 5 123 969
- US-A- 5 405 463
- US-A- 5 582 658
- US-A- 5 690 755
- PATENT ABSTRACTS OF JAPAN vol. 009, no. 184 (C-294), 30 July 1985 (1985-07-30) -& JP 60 052528 A (KAWASAKI SEITETSU KK), 25 March 1985 (1985-03-25)
- PATENT ABSTRACTS OF JAPAN vol. 009, no. 306 (C-317), 3 December 1985 (1985-12-03) -& JP 60 145355 A (KAWASAKI SEITETSU KK), 31 July 1985 (1985-07-31)
- PATENT ABSTRACTS OF JAPAN vol. 1995, no. 07, 31 August 1995 (1995-08-31) -& JP 07 090482 A (KAWASAKI STEEL CORP), 4 April 1995 (1995-04-04)

## Description

### Technical Field

The present invention relates to a cold-rolled steel sheet, which is suitable as raw material steel sheet for molded products such as building members, mechanical structural parts, automobile structural parts, etc., which is used at positions required to have structural strength, particularly, strength and/or stiffness in deformation, and which is subjected to heat treatment for increasing strength after processing such as pressing or the like, and a method of producing these steel sheet.
1. In the present invention, "excellent strain age hardenability" means that in aging under conditions of holding at a temperature of 170°C for 20 min. after pre-deformation with a tensile strain of 5%, the increment in deformation stress (represented by the amount of BH = yield stress after aging - pre-deformation stress before aging) after aging is 80 MPa or more, and the increment in tensile strength (represented by ΔTS = tensile strength after aging - tensile strength before pre-deformation) after strain aging (pre-deformation + aging) is 40 MPa or more.

### Background Art

In producing a press-molded product of a thin steel sheet, a process of coating and baking at lower than 200°C is used as a method in which a material having low deformation stress before press forming to facilitate press forming, and then hardened after press forming to increase the strength of a part. As a steel sheet for such coating and baking, a BH steel sheet has been developed.

For example, Japanese Unexamined Patent Application Publication No. 55-141526 discloses a method in which Nb is added according to the contents of C, N and Al of steel, Nb/(dissolved C + dissolved N) by at% is limited in a specified range, and the cooling rate after annealing is controlled to adjust dissolved C and dissolved N in a steel sheet. Also, Japanese Examined Patent Application Publication No. 61-45689 discloses a method in which baking hardenability is improved by adding Ti and Nb.

However, in order to improve deep drawability, strength of the raw material sheets of the above-described steel sheets is decreased, and thus the steel sheets are not always sufficient as structural materials.

Japanese Unexamined Patent Application Publication No. 5-25549 discloses a method in which baking hardenability is improved by adding W, Cr and Mo to steel singly or in a combination.

In the above-described conventional techniques, strength is increased by bake-hardening due to the functions of small amounts of dissolved C and dissolved N in a steel sheet, and it is well known that a BH(Bake-Hardening) steel sheet is used for increasing only the yield strength of a material, not for increasing tensile strength. Therefore, the conventional techniques have only the effect of increasing the deformation start stress of a part, and the effect of increasing stress (tensile strength after forming) required for deformation over the entire deformation region from the deformation start to the deformation end is not said to be sufficient.

As a cold-rolled steel sheet having tensile strength increased after forming, for example, Japanese Unexamined Patent Application Publication No. 10-310847 discloses an alloying ho-dip galvanized steel sheet having tensile strength increased by 60 MPa or more by heat treatment in the temperature region of 200 to 450°C.

This steel sheet contains, by mass%, 0.01 to 0.08% of C, and 0.01 to 3.0% of Mn, and at least one of W, Cr, and Mo in a total of 0.05 to 3.0%, and further contains at least one of 0.005 to 0.1% of Ti, 0.005 to 0.1% of Nb and 0.005 to 0.1% of V according to demand, and the microstructure of the steel is composed of ferrite or mainly composed of ferrite.

However, this technique comprises forming a fine carbide in the steel sheet by heat treatment after forming to effectively propagate a dislocation of stress applied during pressing, thereby increasing the amount of strain. Therefore, heat treatment must be performed in the temperature range of 220 to 370°C. There is thus the problem of a necessary heat treatment temperature higher than general bake-hardening temperatures.

Furthermore, it is a very important problem that the body weight of an automobile is decreased in relation to the recent regulation of exhaust gases due to global environmental problems. In order to decrease the body weight of an automobile, it is effective to increase the strength of the used steel sheet, i.e., use a high-tensile-strength steel sheet, thinning the steel sheet used.

An automobile part using a high-tensile-strength thin steel sheet must exhibit a sufficient property according to its function. The property depends upon the part, and examples of the property include dent resistance, static strength against deformation such as bending, twisting, or the like, fatigue resistance, impact resistance, etc. Namely, the high-tensile-strength steel sheet used for an automobile part is required to be excellent in such a property after forming. The properties are related to the strength of a steel sheet after forming, and thus the lower limit of strength of the high-tensile-strength steel sheet used must be set for achieving thinning.

On the other hand, in the process for forming an automobile part, a steel sheet is press-molded. If the steel sheet has excessively high strength in press forming, the steel sheet causes the following problems: (1) deteriorating shape fixability; (2) deteriorating ductility to cause cracking, necking, or the like during forming; and (3) deteriorating dent resistance (resistance to a dent produced by a local compressive load) when the sheet thickness is decreased. These problems thus inhibit the extension of application of the high-tensile-strength steel sheet to automobile bodies.

As a means for overcoming the problems, a steel sheet composed of ultra-low-carbon steel is known as a raw material, for example, for a cold-rolled steel sheet for an external sheet panel, in which the content of C finally remaining in a solid solution state is controlled to an appropriate range. This type of steel sheet is kept soft during press forming to ensure shape fixability and ductility, and its yield stress is increased by utilizing the strain aging phenomenon which occurs in the step of coating and baking at 170°C for about 20 minutes after press forming, to ensure dent resistance. This steel sheet is soft during press forming because C is dissolved in steel, while dissolved C is fixed to a dislocation introduced in press forming in the coating and baking step after press forming to increase the yield stress.

However, in this type of steel sheet, the increase in yield stress due to strain age hardening is kept down from the viewpoint of prevention of the occurrence of stretcher strain causing a surface defect. This causes the fault that the steel sheet actually less contributes to a reduction in weight of a part.

On the other hand, a steel sheet composed of dissolved N to further increase the amount of bake-hardening, and a steel sheet provided with a composite structure composed of ferrite and martensite to further improve baking hardenability have been proposed for applications in which the appearance is not so important.

For example, Japanese Unexamined Patent Application Publication No. 60-52528 discloses a method of producing a high-strength steel thin sheet having good ductility and spot weldability, in which steel containing 0.02 to 0.15% of C, 0.8 to 3.5% of Mn, 0.02 to 0.15% of P, 0.10% or less of Al, and 0.005 to 0.025% of N is hot-rolled by coiling at a temperature of 550°C or less, cold-rolled, and then annealed by controlled cooling and heat treatment. A steel sheet produced by the technique disclosed in Japanese Unexamined Patent Application Publication No. 60-52528 has a mixed structure comprising a low-temperature transformation product phase mainly composed of ferrite and martensite, and having excellent ductility, and high strength is achieved by utilizing strain aging due to positively added N during coating baking.

Although the technique disclosed in Japanese Unexamined Patent Application Publication No. 60-52528 greatly increases yield stress YS due to strain age hardening, the technique less increases tensile strength TS. Also, this technique causes large variations in the increment in yield stress YS to cause large variations in mechanical properties, and thus it cannot be expected that a steel sheet can be sufficiently thinned for contributing to a reduction in weight of an automobile part, which is currently demanded.

Japanese Examined Patent Application Publication No. 5-24979 discloses a high-tensile-strength cold-rolled steel thin sheet having baking hardenability which has a composition comprising 0.08 to 0.20% of C, 1.5 to 3.5% of Mn, and the balance composed of Fe and inevitable impurities, and a structure composed of homogeneous bainite containing 5% or less of ferrite, or bainite partially containing martensite. The cold-rolled steel sheet disclosed in Japanese Examined Patent Application Publication No. 5-24979 is produced by quenching in the temperature range of 200 to 400°C in the cooling process after continuous annealing, and then slowly cooling to obtain a structure mainly composed of bainite and having a large amount of bake-hardening which is not obtained by a conventional method.

However, in the steel sheet disclosed in Japanese Examined Patent Application Publication No. 5-24979, yield strength is increased after coating and baking to obtain a large amount of bake-hardening which is not obtained a conventional method, while tensile strength cannot be increased. Therefore, in application to a strength member, improvements in fatigue resistance and impact resistance after forming cannot be expected. Therefore, there is a problem in which the steel sheet cannot be used for applications greatly required to have fatigue resistance and impact resistance, etc.

Also, Japanese Examined Patent Application Publication No. 61-12008 discloses a method of producing a high tensile strength steel sheet having a high r value. This method is characterized by annealing ultra-low-C steel used as a raw material in a ferrite-austenite coexistence region after cold rolling. However, the resultant steel sheet has a high r value and a high degree of baking hardenability (BH property), but the obtained BH amount is about 60 MPa at most. Also, the yield point of the steel sheet is increased after strain aging, but TS is not increased, thereby causing the problem of limiting application to parts.

Furthermore, the above-described steel sheet exhibits excellent strength after coating and baking in a simple tensile test, but produces large variations in strength during plastic deformation under actual pressing conditions. Therefore, it cannot be said that the steel sheet is sufficiently applied to parts required to have reliability.

With respect of a hot-rolled steel sheet among coating baked steel sheets for press molded products, for example, Japanese Examined Patent Application Publication No. 8-23048 discloses a method of producing a hot-rolled steel sheet which is soft during processing, and has tensile strength increased by coating and baking after processing to be effective to improve fatigue resistance.

In this technique, steel contains 0.02 to 0.13 mass % of C, and 0.0080 to 0.0250 mass % of N, and the finisher deliver temperature and the coiling temperature are controlled to leave a large amount of dissolved N in the steel, thereby forming a composite structure as a metal structure mainly composed of ferrite and martensite. Therefore, an increase of 100 MPa or more in tensile strength is achieved at the heat treatment temperature of 170°C after forming.

Japanese Unexamined Patent Application Publication No. 10-183301 discloses a hot-rolled steel sheet having excellent baking hardenability and natural aging resistance, in which the C and N contents are limited to 0.01 to 0.12 mass % and 0.0001 to 0.01 mass %, respectively, and the average crystal grain diameter is controlled to 8 µm or less to ensure a BH amount of as high as 80 MPa or more, and suppress the AI amount to 45 MPa or less.

However, this steel sheet is a hot-rolled sheet, and is thus difficult to obtain a high r value because the ferrite aggregation texture is made random due to austeniste-ferrite transformation. Therefore, the steel sheet cannot be said to have sufficient deep drawability.

Furthermore, even if the hot-rolled steel sheet obtained by this technique is used as a starting material for cold rolling and recrystallization annealing, the increase in tensile strength obtained after forming and heat treatment is not always equivalent to a hot-rolled steel sheet, and a BH amount of as high as 80 MPa or more cannot be always obtained. This is because the microstructure of the cold -rolled steel becomes different from that of hot-rolled one due to cold rolling and recrystallization annealing, and strain greatly accumulates during cold rolling to easily form a carbide, a nitride or a carbonitride, thereby changing the states of dissolved C and dissolved N.

Further, prior art EP 0 943 696 A1 discloses steel plates for drum cans and a method of manufacturing such steel plates. The steel sheet known from this prior art document has a composition comprising C, Si, Mn, P, S, Al and N as mandatory elements. According to the teaching of this prior art document, the structure of said steel sheet is not particularly limited.

In consideration of the above-described present conditions, it is an object of the present invention to solve the above problems of the conventional techniques and provide a high-tensile-strength cold-rolled steel sheet which is suitable for automobile parts required to have high moldability, softness and high moldability, and stable material properties, and which can easily be molded to an automobile part having a complicated shape without producing shape defects such as spring back, twisting, and curving, and cracking, etc., and which has sufficient strength as an automobile part after heat treatment of a molded automobile part to permit sufficient contribution to a reduction in body weight of an automobile, a high r value of 1.2 or more, and excellent strain age hardenability. A further object of the present invention is to provide an industrial production method capable of producing the steel sheet at low cost without disturbing its shape.

### Disclosure of Invention

In order to achieve the objects, the inventors produced various steel sheets having different compositions under various production conditions, and experimentally evaluated various material properties. As a result, it was found that both moldability and hardenability after forming can be improved by using as a strengthening element N, which has not be positively used before in a field requiring high processability, and effectively using the great strain age hardening phenomenon manifested by the action of the strengthening element.

The inventors also found that in order to advantageously use the strain age hardening phenomenon due to N, the strain age hardening phenomenon due to N must be advantageously combined with a condition for coating and baking an automobile, or further positively combined with a heat treatment condition after forming. It was thus found to be effective to appropriately control the hot rolling condition, the cold rolling and the cold rolling annealing condition to control the microstructure of a steel sheet and the amount of dissolved N in certain ranges. It was also found that in order to stably manifest the strain age hardening phenomenon due to N, it is important to control the Al content of the composition according to the N content.

The inventors further found that in order to obtain a high r value, the C content is decreased, continuous annealing is performed in the ferrite-austenite two-phase temperature region, and subsequent cooling is controlled to form a structure containing an acicular ferrite phase at an area ratio of 5% or more in the ferrite phase. Such a combination of the microstructure and the appropriate amount of dissolved N was found to enable the achievement of a cold-rolled steel sheet having a high r value, excellent press moldability, and excellent strain age hardenability. This was also found to permit sufficient use of N without causing the problem of natural aging deterioration, which is the problem of a conventional bake-hardening steel sheet.

Namely, the inventors found that by suing N as a strengthening element, controlling the Al content according to the N content in an appropriate range, and appropriately controlling the hot rolling condition and the cold rolling annealing condition to appropriately control the microstructure and dissolved N, it is possible to obtain a steel sheet having a high r value and excellent moldability as compared with conventional solid-solution strengthening-type C-Mn steel sheets and precipitation strengthening-type steel sheets, and strain age hardenability, which is not possessed by the conventional steel sheets.

A steel sheet of the present invention exhibits higher strength after coating and baking in a simple tensile test, as compared with a conventional steel sheet, and exhibits small variations in strength in plastic deformation under actual pressing conditions and stable part strength, thereby enabling application to parts required to have reliability. For example, a portion where large strain is applied to decrease the thickness has higher hardenability than other portions, and is considered homogeneous when being evaluated based on a surcharge load ability of (thickness) x (strength), thereby stabilizing strength as a part.

As a result of further intensive research for achieving the objects, the inventors found the following:
1) In order to increase tensile strength after forming and heat treatment, a new dislocation must be introduced for progressing tensile deformation. The movement of the dislocation introduced by pre-deformation must be prevented by interaction between the dislocation introduced by forming and an interstitial element or a precipitate even when upper yield stress is attained.
2) In order to obtain the above interaction by forming a carbide, a nitride or a carbonitride of W, Cr, Mo, Ti, Nb, A1 or the like, the heat treatment temperature after forming must be increased to 200°C or more. Therefore, it is more advantageous to positively use the interstitial element or a Fe carbide or Fe nitride because the heat treatment temperature after forming is decreased.
3) Of interstitial elements, dissolved N has the higher interaction with a dislocation introduced by forming than dissolved C even when the heat treatment temperature after forming is decreased, and thus a dislocation introduced by pre-deformation less moves when upper yield stress is attained.
4) Although dissolved N is present in crystal grains and crystal grain boundaries in steel, the increase in strength after forming and heat treatment increases as the area of the crystal grain boundaries increases. Namely, the smaller crystal grain diameter is advantageous.
5) In order to increase the crystal grain boundary area, it is advantageous to add a combination of Nb and B and cool immediately after the end of hot rolling, suppressing normal grain growth of ferrite grains after the end of hot rolling and suppressing grain growth by recrystallization annealing after cold rolling.

The present invention has been achieved based on the above findings. The findings were obtained from the experiment described below. Experiment 1

A sheet bar (thickness: 30 mm) having a composition containing, by mass %, 0.0015% of C, 0.0010% of B, 0.015 of Si, 0.5% of Mn, 0.03% of P, 0.08% of S and 0.011% of N, 0.005 to 0.05% of Nb and 0.005 to 0.03% of Al, and the balance composed of Fe and inevitable impurities was uniformly heated at 1150°C, hot-rolled by three passes so that the temperature of the final pass was 900°C higher than the Ar₃ transformation point, and then cooled with water for 0.1 second. Then, the sheet bar was subjected to heat treatment corresponding to coiling at 500°C for 1 hour.

The thus-obtained hot-rolled sheet having a thickness of 4 mm was cold-rolled with a rolling reduction ratio of 82,5%, recrystallized and annealed at 800°C for 40 seconds, and then temper-rolled with a rolling reduction ratio of 0.8%. Then, a tensile test specimen of JIS No. 5 was obtained from the resultant cold-rolled sheet in the rolling direction, and tensile strength was measured with a strain rate of 0.02/s by using a general tensile testing machine. Also, tensile strain of 10% was applied to a tensile test specimen of JIS No. 5 separately obtained from the cold-rolled sheet in the rolling direction, and then the specimen was subjected to a normal tensile test after heat treatment at 120°C for 20 minutes. The difference between the tensile strength of the specimen obtained from the cold-rolled sheet and the tensile strength of the specimen heat treated at 120°C for 20 minutes after application of 10% tensile strain was considered as the increase in tensile strength after forming (ΔTS).

Fig. 1 shows the results of measurement of the relation between the steel compositions (N% - 14/93•Nb% - 14/27•Al% - 14/11•B%) and ΔTS.

The figure indicates that ΔTS becomes 60 MPa or more when the value of (N% - 14/93•Nb% - 14/27•Al% - 14/11•B%) satisfies 0.0015 mass %. Experiment 2

A sheet bar (thickness: 30 mm) having a composition containing, by mass %, 0.0010% of C, 0.02 of Si, 0.6% of Mn, 0.01% of P, 0.009% of S and 0.012% of N, 0.01% of Al, 0.015% of Nb, 0.00005 to 0.0025% of B, and the balance composed of Fe and inevitable impurities was uniformly heated at 1100°C, hot-rolled by three passes so that the temperature of the final pass was 920°C higher than the Ar₃ transformation point, and then cooled with water for 0.1 second. Then, the sheet bar was subjected to heat treatment corresponding to coiling at 450°C for 1 hour.

The thus-obtained hot-rolled sheet having a thickness of 4 mm was cold-rolled with a rolling reduction ratio of 82,5%, recrystallized and annealed at 820°C for 40 seconds, and then temper-rolled with a rolling reduction ratio of 0.8%. Then, a tensile test specimen of JIS No. 5 was obtained from the resultant cold-rolled sheet in the rolling direction, and tensile strength was measured with a strain rate of 0.02/s by using a general tensile testing machine. Also, tensile strain of 10% was applied to a tensile test specimen of JIS No. 5 separately obtained from the cold-rolled sheet in the rolling direction, and then the specimen was subjected to a normal tensile test after heat treatment at 120°C for 20 minutes.

Fig. 2 shows the results of measurement of the relation between the B content of steel and ΔTS. This figure indicates that with a B content of 0.0005 to 0.0015 mass %, a high ΔTS of 60 MPa or more can be obtained.

As a result of observation of the microstructure, it was also found that by adding a combination of Nb and B to make fine crystal grains, a high ΔTS can be obtained.

Namely, with a B content of less than 0.0005 mass %, the effect of making fine crystal grains by adding a combination with Nb is small. On the other hand, with a B content of over 0.0015 mass %, the amount of B segregated in the grain boundaries and the vicinities thereof is increased to decrease the amount of effective dissolved N because of the strong interaction between B atoms and N atoms, thereby possibly decreasing ΔTS.

### Experiment 3

A sheet bar (thickness: 30 mm) of each of steel A having a composition containing, by mass %, 0.0010% of C, 0.012% of N, 0.0010% of B, 0.01% of Si, 0.5% of Mn, 0.03% of P, 0.008% of S, 0.014% of Nb, 0.01% of Al, and the balance composed of Fe and inevitable impurities, and steel B having a composition containing, by mass %, 0.010% of C, 0.0012% of N, 0.0010% of B, 0.01% of Si, 0.5% of Mn, 0.03% of P, 0.008% of S, 0.014% of Nb, 0.01% of Al, and the balance composed of Fe and inevitable impurities was uniformly heated at 1150°C, hot-rolled by three passes so that the temperature of the final pass was 910°C higher than the Ar₃ transformation point, and then cooled with a gas for 0.1 second. Then, each of the sheet bars was subjected to heat treatment corresponding to coiling at 600°C for 1 hour.

Each of the thus-obtained hot-rolled sheets having a thickness of 4 mm was cold-rolled with a rolling reduction ratio of 82,5%, recrystallized and annealed at 880°C for 40 seconds, and then temper-rolled with a rolling reduction ratio of 0.8%.

Then, a tensile test specimen of JIS No. 5 was obtained from each of the resultant cold-rolled sheets in the rolling direction, and tensile strength was measured with a strain rate of 0.02/s by using a general tensile testing machine. Also, tensile strain of 10% was applied to a tensile test specimen of JIS No. 5 separately obtained from each of the cold-rolled sheets in the rolling direction, and then the specimen was subjected to a normal tensile test after heat treatment at various temperatures for 20 minutes.

Fig. 3 shows the results of measurement of the influence of the heat treatment temperature after forming on ΔTS. This figure indicates that in the relatively low temperature region of heat treatment temperatures of 200°C or less after forming, the ultra-low carbon steel A having a high N content exhibits higher ΔTS than the semi-ultra low carbon steel B having a low N content, and while in the high temperature region, both steel materials exhibit substantially the same ΔTS. There experimental results reveal that in order to ensure ΔTS in the low temperature region, it is effective to use dissolved N.

Fig. 4 shows the results of measurement of the influences of the crystal grain diameter d and steel compositions (N% - 14/93•Nb% - 14/27•Al% - 14/11•B%) on a decrease (ΔEl) in elongation by natural aging and an increase in tensile strength (ΔTS) after forming. The decrease (ΔEl) in elongation was evaluated by the difference between the total elongation measured with the test specimen of JIS NO. 5 obtained from each of the cold-rolled sheets in the rolling direction, and the total elongation measured with the separately obtained test specimen after holding at 100°C for 8 hours for accelerating natural aging.

Fig. 4 indicates that when the value of (N% - 14/93•Nb% - 14/27•Al% - 14/11•B%) is 0.0015 mass % or more, and the crystal grain diameter d is 20 µm or less, both high ΔTS and low ΔEl can be achieved.

### Experiment 4

A sheet bar of steel containing 0.0015% of C, 0.30 of Si, 0.8% of Mn, 0.03% of P, 0.005% of S and 0.012%.of N, and 0.02 to 0.08% of Al was uniformly heated at 1050°C, hot-rolled by seven passes so that the temperature of the final pass was 670°C, and then recrystallized and annealed at 700°C for 5 hours. The thus-obtained hot-rolled sheet having a thickness of 4 mm was cold-rolled with a rolling reduction ratio of 82,5%, recrystallized and annealed at 875°C for 40 seconds, and then temper-rolled with a rolling reduction of 0.8%. Then, a tensile test specimen of JIS No. 5 was obtained from the resultant cold-rolled sheet in the rolling direction, and TS x r value and ΔTS were measured with a strain rate of 3 x 10⁻³/s by using a general tensile testing machine. The results are shown in Fig. 5. In this figure, when N/Al ≥ 0.03 is satisfied, TS x r value ≥ 750 and ΔTS ≥ 40 MPa are achieved. It was also confirmed that when N/Al ≥ 0.03, BH ≥ 80 MPa is attained. Experiment 5

A sheet bar of steel containing 0.0015% of C, 0.0010% of B, 0.01 of Si, 0.5% of Mn, 0.03% of P, 0.008% of S and 0.011% of N, 0.005 to 0.05% of Nb, and 0.005 to 0.03% of A1 was uniformly heated at 1000°C, hot-rolled by seven passes so that the temperature of the final pass was 650°C, and then recrystallized and annealed at 800°C for 60 seconds. The thus-obtained hot-rolled sheet having a thickness of 4 mm was cold-rolled with a rolling reduction ratio of 82,5%, recrystallized and annealing at 880°C for 40 seconds, and then temper-rolled with a rolling reduction ratio of 0.8%. Then, a tensile test specimen of JIS No. 5 was obtained from the resultant cold-rolled sheet in the rolling direction, and TS x r value, BH and ΔTS were measured with a strain rate of 3 x 10⁻³/s by using a general tensile testing machine. The relations between the measured values and N/(Al+Nb+B) are shown in Fig. 5. In this experiment, steel containing 0.005 to 0.05% of Nb and 0.0010% of B was used. This figure indicates that in the range of N/(A1+Nb+B) ≥ 0.30, BH ≥ 80 MPa, ΔTS ≥ 60 MPa, and TS x r value ≥ 850 are achieved.

### Experiment 6

A sheet bar of steel containing 0.0010% of C, 0.02 of Si, 0.6% of Mn, 0.01% of P, 0.009% of S and 0.015% of N, 0.01% of Al, 0.015% of Nb and 0.0001 to 0.0025% of B was uniformly heated at 1050°C, hot-rolled by seven passes so that the temperature of the final pass was 680°C, and then recrystallized and annealed at 850°C for 5 hours. The thus-obtained hot-rolled sheet having a thickness of 4 mm was cold-rolled with a rolling reduction ratio of 82,5%, recrystallized and annealed at 880°C for 40 seconds, and then temper-rolled with a rolling reduction ratio of 0.8%. Then, a tensile test specimen of JIS No. 5 was obtained from the resultant cold-rolled sheet in the rolling direction, and TS x r value, BH and ΔTS were measured with a strain rate of 3 x 10⁻³/s by using a general tensile testing machine. The relations between the measured values and the B content are shown in Fig. 6.

This figure indicates that in the B content range of 0.0003 to 0.0015%, BH ≥ 80 MPa, ΔTS ≥ 60 MPa, which is higher than the case of B < 0.0003%, and TS x r value ≥ 850 are achieved. As a result of observation of the microstructure, it was also confirmed that in this B range, crystal grains are significantly made fine.

The results shown in Figs. 5 and 6 indicate that in the range of N/(Al+Nb+B) ≥ 0.30 wherein B ≥ 0.0003%, the crystal grains are further made fine by combining Nb, and ΔTS and the level of TS x r value are further improved. When B < 0.0003%, the effect of making fine crystal grains by combining Nb is not exhibited. On the other hand, when B > 0.0015%, properties further deteriorate. This is possibly due to the fact that the amount of B segregated in the grain boundaries and the vicinities thereof is increased to decrease the amount of effective dissolved N due to the strong interaction between B and N atoms. The same research as described above was carried out for the case in which Ti and V were added in place of Nb, and it was confirmed that the same effect as Nb could be obtained. The present invention has been achieved based on the above-described findings, and the gist of the invention was follows.

According to the present invention, a high-tensile-strength cold-rolled steel sheet as defined in claim 1 is provided in order to solve the above object. In order to solve said further object a method as defined in claim 3 is provided prefered embodiments of the inventive steel sheet and method are subject to the dependent claims.

### Brief Description of the Drawings

Fig. 1 shows the relation between steel compositions (N% - 14/93•Nb% - 14/27•Al% - 14/11•B%) and the increase in tensile strength (ΔTS) after forming.
Fig. 2 shows the relation between the B content and ΔTS of steel containing a combination Nb and B.
Fig. 3 shows comparison of the difference in increase in tensile strength by heat treatment after forming in a low temperature region between steel B (conventional steel) containing a large amount of dissolved C and steel A containing a large amount of dissolved N.
Fig. 4 shows the influence of the crystal grain diameter d and steel compositions (N% - 14/93•Nb% - 14/27•Al% - 14/11•B%) on the decrease in elongation (ΔEl) due to natural aging and the increase in tensile strength (ΔTS) after forming.
Fig. 5 shows the relations between Ts x r value, BH, ΔTS and N/(Al+Nb+B).
Fig. 6 shows the relations between Ts x r value, BH, ΔTS and the B amount.

### Best Mode for Carrying Out the Invention

Description will now be made of the reasons for limiting compositions to the ranges below in accordance with an embodiment of the present invention.

### C: 0.025 to 0.15%

C is an element for increasing the strength of a steel sheet, and 0.025% or more of C must be contained for controlling the structure to a homogeneous fine structure, which is an important requirement of the present invention, and ensuring a sufficient amount of a martensite phase. With a C content of over 0.15%, the ratio of the carbide in the steel sheet is excessively increased to significantly deteriorate ductility and moldability. With a C content of over 0.15%, there is the more important problem of significantly deteriorating spot weldability and arc weldability. Therefore, the C content is limited in the range of 0.025 to 0.15%. From the viewpoint of improvement in moldability, the C content is preferably 0.08% or less. Particularly, when good ductility is required, the C content is preferably 0.05% or less.

### Si: 1.0% or less

Si is a useful component capable of increasing the strength of the steel sheet without significantly deteriorating ductility of steel. The Si content is preferably 0.005% or more, and more preferably 0.10% or more. On the other hand, Si is an element which greatly changes the transformation point during hot rolling to cause difficulties in ensuring quality and the shape, or adversely affects surface properties, chemical conversion properties, and the like, particularly the beauty of the surface of the steel sheet, and adversely affects plating properties. In the present invention, therefore, the Si content is limited to 1.0% or less. However, the above-described adverse effects can be kept down as long as Si is 1.0% or less. Particularly, in applications required for the steel sheet to have a low level of strength and, particularly, surface beauty, Si is preferably 0.5% or less.

### Mn: 2.0% or less

Mn is an element effective to prevent hot cracking with S, and Mn is preferably added according to the amount of S contained. Mn also has the great effect of making fine crystal grains, and is preferably added for improving material properties. Furthermore, Mn is an element effective to stably form martensite during rapid cooling after continuous annealing. In order to stably fix S, the Mn content is preferably 0.2% or more. Mn is also an element for increasing the strength of the steel sheet, and is preferably added in an amount of 1.2% or more when a strength TS of over 500 MPa is required. The Mn content is more preferably 1.5% or more.

With the Mn content increased to this level, there is the advantage that variations in the mechanical properties of the steel sheet with respect to variations in the hot-rolling conditions, particularly strain age hardenability, are significantly improved. However, with the excessively high Mn content of over 2.0%, a high r value, which is an important requirement of the present invention, cannot be easily obtained, and ductility significantly deteriorates. Therefore, the Mn content is limited to 2.0% or less. In applications required to have good corrosion resistance and moldability, the Mn content is preferably 1.7% or less.

### P: 0.08% or less

P is a useful element as a solid solution strengthening element for steel, and is preferably added in an amount of 0.001% or more, and more preferably 0.015% or more, from the viewpoint of an increase in strength. On the other hand, when P is excessively added, steel is embrittled, and stretch-flanging properties of the steel sheet deteriorate. Also, P is liable to strongly segregate in steel, thereby causing embrittlement of a weld. Therefore, P is limited to 0.08% or less. In applications in which elongated flange processability and weld toughness are considered as important, P is preferably 0.04% or less.

### S: 0.02% or less

S is present as an inclusion in the steel sheet, decreases ductility of the steel sheet, and causes deterioration in corrosion resistance. Therefore, the Si content is as low as possible, and in the present invention, the S content is limited to 0.02% or less. Particularly, in applications required to have good processability, S is preferably 0.015% or less. Particularly, in applications required to have excellent stretch-flanging properties, S is preferably 0.008% or less. Although the detailed mechanism is not known, in order to stably maintain the strain age hardenability of the steel sheet in a high level, it is effective to decrease the S content to 0.008% or less.

### Al: 0.02% or less

Al is an element functioning as a deoxidization for improving cleanliness of steel, and making fine the structure of the steel sheet. In the present invention, the Al content is preferably 0.001% or more. In the present invention, dissolved N is used as a strengthening element, but aluminum killed steel containing Al in a suitable range has mechanical properties superior to those of conventional rimmed steel not containing Al. On the other hand, with an excessively high Al content, the surface properties of the steel sheet deteriorate, and the amount of dissolved N is significantly decreased to cause difficulties in obtaining a large amount of strain age hardening, which is the main object of the present invention. Therefore, in the present invention, Al is limited to 0.02% or less. From the viewpoint of stability of material properties, Al is more preferably 0.001 to 0.015%. Although a decrease in the Al content possibly causes coarsening of crystal grains, in the present invention, the amounts of other alloy elements are appropriately determined to appropriately set the annealing conditions, thereby effective preventing coarsening.

### N: 0.0050 to 0.0250%

N is an element for increasing the strength of the steel sheet by solid solution strengthening and strain age hardening, and in the present invention, N is the most important element. In the present invention, an appropriate amount of N is contained, the Al content is controlled to the appropriate value, and production conditions such as the hot-rolling conditions, and the annealing conditions are controlled to ensure necessary and sufficient dissolved N in a cold-rolled product or a coated product. This exhibits the sufficient effect of increasing strength (yield stress and tensile strength) by solid solution strengthening and strain age hardening, to stably obtain the target values of the mechanical properties of the steel sheet of the present invention, such as a tensile strength of 440 MPa or more, an amount (BH amount) of bake-hardening of 80 MPa or more, and an increase is tensile strength ΔTS of 40 MPa or more after strain aging. Since N also has the function to decrease the transformation point, N is effective for rolling of a thin material for which rolling at a temperature greatly over the transformation point is undesirable.

With a N content of less than 0.0050%, the effect of increasing strength is less stably exhibited, while with a N content of over 0.0250%, the rate of occurrence of internal defects in the steel sheet is increased, and slab cracking frequently occurs during continuous casting. Therefore, N is limited to the range of 0.0050 to 0.0250%. From the viewpoint of improvement in stability of material properties and yield over the entire production process, N is preferably in the range of 0.0070 to 0.0170%. With the N amount in the range of the present invention, there is no adverse effect on weldability, and the like.

### Dissolved N: 0.0010% or more

In order to ensure sufficient strength of a cold-rolled product, and effectively exhibit strain age hardening with N, it is necessary that the content of dissolved N (solid solution N) in the steel sheet is at least 0.0010% or more.

The amount of dissolved N is determined by subtracting the amount of precipitated N from the total N amount of steel. As a result of comparison research of various methods, the inventors found that electrolytic extraction analysis using constant-potential electrolysis is effective as the method of analyzing the amount of precipitated N. As the method of dissolving ferrite used for extraction analysis, an acid digestion method, a halogen method, or an electrolysis method can be used. Of these methods, the electrolysis method can stably dissolve only ferrite without decomposing very unstable precipitates such as a carbide, a nitride, etc. As the electrolyte, an acetyl-acetone system is used for electrolysis at a constant potential. In the present invention, the results of measurement of the amount of precipitated N by constant-potential electrolysis showed best correspondence with changes in actual material properties.

Therefore, in the present invention, the residue after extraction by constant-potential electrolysis is chemically analyzed to determine the amount of N in the residue. The thus-determined value is considered as the amount of precipitated N.

In order to obtain higher BH and ΔTS, the amount of dissolved N is preferably 0.0020% or more, more preferably 0.0020% or more. In order to obtain further high values, the amount of dissolved N is preferably 0.0030% or more. Although the upper limit of the amount of dissolved N is not limited, the mechanical properties less deteriorate even when the all amount of N added remains.

### N/Al (the content ratio of N to Al): 0.3 or more

In order to cause 0.0010% or more of dissolved N to stably remain in a product state, the amount of Al which is an element for strongly fixing N, must be limited. As a result of research of steel sheets in which the combination of the N content (0.0050 to 0.0250%) and the Al content (0.02% or less) were widely changed in the composition range of the present invention, it was found that with N/Al of 0.3 or more, the amount of dissolved N of a cold-rolled product or coated product can be stably set to 0.0010% or more. Therefore, N/Al is limited to 0.3 or more.

In the present invention, the above component preferably further contains at least one of the following groups d to g:
Group d: at least one of Cu, Ni, Cr and Mo in a total of 1.0% or less;
Group e:' at least one of Nb, Ti and V in a total of 0.1% or less;
Group f: 0.00305 of B; and
Group g: one or both of Ca and REM in a total of 0.0010 to 0.010%.

Elements of group d: Cu, Ni, Cr and Mo are all contribute to an increase in strength of the steel sheet, and can be contained singly or in a combination according to demand. The effect is recognized by containing 0.005% or more each of Cu, Ni, Cr and Mo. However, with an excessively high content, deformation resistance in hot rolling at elevated temperatures is increased, or chemical conversion properties and surface treatment properties in a wide sense deteriorate, and a welded portion is hardened to deteriorate weld moldability. Also, the r value is liable to decrease. Therefore, the elements of group a are preferably contained in a total of 1.0% or less. With a Mo content of 0.05% or more, the r value is significantly decreased in some cases. In the present invention, therefore, the Mo content is preferably limited to less than 0.05%.

Elements of group e: All of Nb, Ti and V are elements contributing refinement and homegenization of crystal grains, and may be added singly or in a combination according to demand. The effect can be recognized by containing 0.005% or more each of Nb, Ti and V. However, with an excessively high content, deformation resistance in hot rolling at elevated temperatures is increased, or chemical conversion properties and surface treatment properties in a wide sense deteriorate. Therefore, the elements in group b are preferably contained at a total of 0.1% or less.

Elements of group f: B is an element having the effect of improving hardenability of steel, and can be contained for increasing the fraction of a low-temperature transformation phase other than the ferrite phase to increase strength of steel according to demand. This effect is recognized with a B content of 0.0005% or more. However, with an excessively high B content, deformability at elevated temperatures in hot rolling deteriorates to produce BN, decreasing the amount of dissolved N. Therefore, the B content is preferably 0.0030% or less.

Elements in group g: Both Ca and REM are elements useful for controlling the form of inclusions. Particularly, when the stretch flanging property is required, these elements are preferably added singly or in a combination. When the total of the elements of group d is less than 0.0010%, the effect of controlling the form of inclusions is insufficient, while when the total exceeds 0.010%, surface defects significantly occur. Therefore, the total of the elements of group d is preferably limited to the range of 0.0010 to 0.010%. This permits improvement in the stretch flanging property without causing surface defects.

The structure of the steel sheet of the present invention is described below.

### Area ratio of ferrite phase: 80% or more

The cold-rolled steel sheet of the present invention is directed to use as an automobile steel sheet required to have some extent of moldability, and has a structure containing the ferrite phase at an area ratio of 80% or more in order to ensure ductility. With the ferrite phase at an area ratio of less than 80%, it is difficult to ensure ductility required for an automobile steel sheet required to have moldability. When good ductility is required, the area ratio of the ferrite phase is preferably 85% or more. In the present invention, "ferrite" means so-called polygonal ferrite in which no strain remains.

### Average crystal grain diameter of ferrite phase: 10 µm or less

In the present invention, the value used as the average crystal grain diameter is a higher value of the value calculated from a photograph of a sectional structure by a quadrature method defined by ASTM, and the nominal value determined by an intercept method defined by ASTM (refer to, for example, Umemoto et al.: Heat Treatment, 24 (1984), p334).

The cold-rolled steel sheet of the present invention maintains a predetermined amount of dissolved N in the product step. However, as a result of experiment and research conducted by the inventors, it was found that variations in strain age hardenability occur in steel sheets containing the same amount of dissolved N, and one of the main causes of the variations is a crystal grain diameter. In the structure of the present invention, in order to stably obtain a high BH amount and ΔTS, the average crystal grain diameter is at least 10 µm or less, and preferably 8 µm or less. Although the detailed mechanism is not known, this is supposed to be related to the segregation and precipitation of alloy elements in the crystal grain boundaries, and the influences of processing and heat history on the segregation and precipitation.

Therefore, in order to achieve stability of strain age hardenability, the average crystal grain diameter of the ferrite phase is 10 µm or less, and preferably 8 µm or less.

In order to ensure ductility of an automobile steel sheet, and stability of strain age hardenability, the structure of the present invention contains the ferrite phase with an average crystal grain diameter of 10 µm or less at an area ratio of 80% or more.

### Area ratio of martensite phase: 2% or more

The cold-rolled steel sheet of the present invention contains the martensite phase as a second phase at an area ratio of 2% or more. The presence of 2% or more of the martensite phase can produce good ductility and a large amount of strain age hardening. Although the detailed mechanism is not known, this effect is supposed to be due to the effective accumulation of strain in the steel sheet due to the presence of the martensite phase during pre-strain processing before aging. Furthermore, the presence of the martensite phase is effective to improve aging deterioration. In order to a good balance between strength and ductility and a low yield ratio, the area ratio of the martensite phase is preferably 5% or more. The presence of the martensite phase at an area ratio of over 20% causes the problem of deteriorating ductility. Therefore, the area ratio of the martensite phase is 2% or more, and preferably 5% to 20%.

Besides the above-described martensite phase, pearlite, bainite, residual austenite are present as second phases without causing any problem. However, in the present invention, it is necessary that the fraction of the ferrite phase is 80% or more, and the fraction of the martensite phase is 2% or more. Therefore, the total area ratios of pearlite, bainiate and residual austenite are limited to less than 18%.

The cold-rolled steel sheet of the present invention, which has the above-described composition and structure, has a tensile strength (TS) of 440 MPa to about 780 MPa, a high r value of 1.2 or more obtained by controlling the aggregation structure of the ferrite base phase, and excellent strain age hardenability. A steel sheet having TS of less than 440 MPa cannot be widely applied to members having structural components. Furthermore, in order to extend the application range, TS is preferably 500 MPa or more. With the r value of less than 1.2, the steel sheet cannot be applied to a wide range of press forming parts. The preferable range of the r value is 1.4 or more.

As described above, in the present invention, "excellent strain age hardenability" means that in aging under conditions of holding at a temperature of 170°C for 20 min. after pre-deformation with a tensile strain of 5%, the increment in deformation stress (represented by the amount of BH = yield stress after aging - pre-deformation stress before aging) after aging is 80 MPa or more, and the increment in tensile strength (represented by ΔTS = tensile strength after aging tensile strength without strain aging) after strain aging (pre-deformation + aging) is 40 MPa or more.

In defining the strain age hardenability, the amount of pre-strain (pre-deformation) is an important factor. As a result of research of the influence of the amount of prestrain on strain age hardenability, the inventors found that (1) the deformation stress in the above-described deformation system can be referred to as an amount of approximately uniaxial strain (tensile strain) except the case of excessive deep drawing, (2) the amount of uniaxial strain of an actual part exceeds 5%, and (3) the strength of a part sufficiently corresponds to the strength (YS and TS) obtained after strain aging with a pre-strain of 5%. In the present invention, based on these findings, the pre-deformation of strain aging is defined to a tensile strain of 5%.

Conventional coating and baking conditions include 170°C and 20 min as standards. When a strain of 5% is applied to the steel sheet of the present invention, which contains a large amount of dissolved N, hardening can be achieved even by aging at low temperature. In other words, the range of aging conditions can be widened. In order to attain a sufficient amount of hardening, generally, retention at a higher temperature for a longer time is advantageous as long as softening does not occurs by over aging.

Specifically, in the steel sheet of the present invention, the lower limit of the heating temperature at which hardening significantly takes place after pre-deformation is about 100°C. On the other hand, with the heating temperature of over 300°C, hardening peaks, thereby causing the tendency to soften and significantly causing thermal strain and temper color. With the retention time of about 30 seconds or more, hardening can be sufficiently achieved at a heating temperature of about 200°C. In order to obtain more stable hardening, the retention time is preferably 60 seconds or more. However, retention for over 20 mines is practically disadvantageous because further hardening cannot be expected, and the production efficiency significantly deteriorates.

Therefore, in the present invention, the conventional coating and baking conditions, i.e., the heating temperature of 170°C and the retention time of 20 minutes, are set as the aging conditions. With the steel sheet of the present invention, hardening can be stably achieved even under the aging conditions of a low heating temperature and a short retention time, which fail to achieve sufficient hardening in a conventional bake-hardening steel sheet. The heating method is not limited, and atmospheric heating with a furnace, which is generally used for coating and baking, and other methods such as induction heating, heating with a nonoxidation flame, a laser, plasma, or the like, etc. can be preferably used.

The strength of an automobile part must be sufficient to resist an external complicated stress load, and thus not only strength in a low strain region but also strength in a high strain region are important for a raw material steel sheet. In consideration of this point, in the steel sheet of the present invention used as a raw material for automobile parts, BH is 80 MPa or more, and ΔTS is 40 MPa or more. More preferably, BH is 100 MPa or more, and ΔTS is 50 MPa or more. In order to further increase BH and TS, the heating temperature in aging may be set to a higher temperature, and/or the retention time may be set to a longer time.

The steel sheet of the present invention has the advantage that when the steel sheet is allowed to stand at room temperature for about one week without heating after forming, an increase in strength of about 40% of that at the time of complete aging can be expected.

The steel sheet of the present invention also has the advantage that even when it is allowed in an unmolded state at room temperature for a long time, aging deterioration (an increase in YS and a decrease in El (elongation)) does not occurs, unlike a conventional aging steel sheet. In order to prevent the occurrence of a trouble in actual press forming, it is necessary that in aging at room temperature for 3 months before press forming, an increase in YS is 30 MPa or less, a decrease in elongation is 2% or less, and a recovery of yield point elongation is 0.2% or less.

In the present invention, the surface of the cold-rolled steel sheet may be coated by hot-dip galvanization or alloying hot-dip galvanization without any problem, and TS, BH and ΔTS are equivalent to those before plating. AS the plating method, electro-galvanization, hot-dip galvanization, alloying hot-dip galvanization, electro-tinning, electric chromium plating, electro-nickeling, and the like may be preferably used.

The method of producing a steel sheet according to the present invention will be described.

The steel sheet of the present invention is basically produced by performing the hot rolling step in which a steel slab having the above-described composition is heated, and then'roughly rolled to form a sheet bar, and the sheet bar is finish-rolled and cooled to form a coiled hot-rolled sheet, the cold rolling step in which the hot-rolled sheet is pickled and cold-rolled to form a cold-rolled sheet, and the cold-rolled sheet annealing step in which the cold-rolled sheet is box-annealing and then continuously annealed.

Although the slab used in the production method of the present invention is preferably produced by a continuous casting method in order to prevent macro-segregation of components, an ingot making method or a thin slab casing method may be used. Alternatively, a conventional method comprising cooling the produced slab to room temperature and then again heating the slab, or an energy-saving process of direct rolling comprising charging a hot slab into a heating furnace without cooling and then rolling it, or rolling directly the slab immediately after slightly keeping it warm may be used without a problem. Particularly, direct rolling is a useful technique for effectively ensuring dissolved N.

Description will be now be made of the reasons for limiting the conditions of the hot rolling step.

Slab heating temperature: 1000°C or more

The slab heating temperature is 1000°C or more in order to ensure a necessary and sufficient amount of dissolved N in an initial state and satisfy the target amount of dissolved N in a product. Since a loss is increased by an increase in the oxide weight, the heating temperature is preferably 1280°C or less.

The slab heated under the above condition is roughly rolled to form a sheet bar. The condition of the rough rolling is not defined, and rough rolling may be performed according to a normal method. However, in order to ensure the amount of dissolved N, rough rolling is preferably performed within a as short time as possible. Then, the sheet bar is finish-rolled to form a hot-rolled sheet.

In the present invention, the adjacent sheet bars are preferably bonded together during the time between rough rolling and finish rolling, and then continuously rolled. As the bonding means, a pressure welding method, a laser welding method, an electron beam welding method, or the like is preferably used.

By continuous rolling, so-called non-stationary portions at the front end and the rear end of a coil (processed material) are removed to permit hot rolling over the entire length and the entire width of the coil (processed material) under stable conditions. This is very effective to improve the sectional shape and dimensions of not only the hot-rolled steel sheet but also the cold-rolled steel sheet. When the steel sheet is cooled on a hot run table after rolling, the shape of the steel sheet can be sufficiently maintained because tension can be always applied.

By continuous rolling, the ends of the coil can be stably passed, and it is thus possible to use lubricating rolling, which cannot be easily applied to ordinary single rolling for each sheet bar because of the problem of continuous rolling processes and biting property. Therefore, the rolling load can be decreased, and at the same time, the surface pressure of the roll can be decreased, thereby increasing the life time of the roll.

In the present invention, at the entrance of a finisher between rough rolling and finish rolling, the temperature distributions of the sheet bar in the width direction and the long direction thereof are preferably made uniform by'using any one or both of a sheet bar edge heater for heating the ends of the sheet bar in the width direction and a sheet bar heater for heating the ends of the sheet bar in the long direction. This can further decrease the variations in material properties of the steel sheet. The sheet bar edge heater and the sheet bar heater are preferably of an induction heating type.

As the procedure of use of the heaters, preferably, the difference in temperature in the width direction is first corrected by the sheet bar edge heater. Although the heating amount depends upon the steel composition, the temperature distribution in the width direction at the finisher entrance is preferably set in the range of about 20°C or less. Next, the difference in temperature in the long direction is corrected by the sheet bar heater. At this time, the heating amount is preferably set so that the temperatures at the ends in the long direction are about 20°C higher than the temperature at the center.

### Finisher delivery temperature: 800°C or more

In order to obtain a homogeneous fine hot-rolled base sheet structure, the finisher deliver temperature FDT is 800°C or more. With a FDT of lower than 800°C, the structure of the steel sheet becomes inhomogeneous, and the processed structure partially remains to leave heterogeneity of the structure after the cold-rolled sheet annealing step. Therefore, the danger of causing various troubles in press forming is increased. When a high coiling temperature is used for avoiding the processed structure from remaining, coarse crystal grains are produced to cause the same troubles as described above. With the high coiling temperature, the amount of dissolved N is significantly decreased to cause difficulties in obtaining a target tensile strength of 440 MPa or more. Therefore, the finisher deliver temperature FDT is 800°C or more. In order to further improve the mechanical properties, the FDT is preferably 820°C or more. Although the upper limit of FDT is not limited, a scale scar significantly occurs at excessively high FDT. The FDT is preferably up to about 1000°C.

Although cooling after finish rolling is not strictly limited, the conditions described below are preferable from the viewpoint of homogeneity in material properties of the steel sheet in the long direction and the width direction thereof. In the present invention, cooling is preferably started immediately after (within 0.5 seconds after) finish rolling, and the mean cooling rate in cooling is preferably 40°C/s or more. By satisfying these conditions, the steel sheet can be rapidly cooled in the high temperature region where AlN precipitates to effectively ensure N in a solid solution state. When the starting time of cooling or the cooling rate does not satisfy the above condition, grain growth excessively proceeds to fail to achieve fine crystal grains, and promote AlN precipitation due to stain energy introduced by rolling. Therefore, the amount of dissolved N tends to decrease, and the structure tends to be made inhomogeneous. In order to ensure homogeneity in material properties and shape, the cooling rate is preferably kept at 300°C/s or less.

### Coiling temperature: 800°C or less

The strength of the steel sheet is liable to increase as the coiling temperature CT decreases. In order to ensure the target tensile strength TS of 440 MPa or more, the CT is 800°C or less. With a CT of less than 200°C, the shape of the steel sheet is readily disturbed to increase the danger of causing troubles in a practical operation, thereby deteriorating homogeneity of material properties. Therefore, the CT is preferably 200°C or more. When the homogeneity of the material properties is required, the CT is preferably 300°C or more, and more preferably 350°C or more. In the present invention, in finish rolling, lubricating rolling may be performed for decreasing the hot rolling load. The lubricating rolling has the effect of further making homogeneous the shape and material properties of the hot-rolled sheet. During the lubricating rolling, the frictional coefficient is preferably in the range of 0.25 to 0.10. By combining lubricating rolling and continuous rolling, the operation of hot rolling is further stabilized.

The hot-rolled sheet subjected to the above-described hot rolling step is then pickled and cold-rolled in the cold rolling step to form a cold-rolled sheet.

The pickling conditions may be the same as conventional known conditions, and are not limited. When the scale of the hot-rolled sheet is extremely small, cold rolling may be immediately after hot rolling without pickling.

The cold rolling conditions may be the same as conventional known conditions, and are not limited. In order to ensure homogeneity of the structure, the reduction ratio of cold rolling is preferably 40% or more. The reasons for limiting the conditions of the cold rolling step are described below.

The cold-rolled sheet is then subjected to the cold-rolled sheet annealing step comprising box annealing and continuous annealing.

Box annealing temperature: the recrystallization temperature to 800°C

In the present invention, the cold-rolled sheet is subjected to box annealing to control the aggregation structure of the ferrite phase as a base. By controlling the aggregation structure of the ferrite phase, the r value of the produced sheet can be increased. By box annealing, the (111) aggregation structure suitable for increasing the r value is readily formed in the produced sheet.

With the box annealing temperature less than the recrystallization temperature, recrystallization is not completed to fail to control the aggregation structure of the ferrite phase, thereby failing to increase the r value. On the other hand, with the box annealing temperature of over 800°C, surface defects significantly occur in the steel-sheet, thereby failing to achieve the initial purpose. Box annealing is preferably performed in an annealing atmosphere containing a nitrogen gas as a main component and 3 to 5% of hydrogen gas. In this case, the heating and cooling rates may be the same as normal box annealing, and are about 30°C/hr. By using 100% hydrogen gas as an annealing atmosphere gas, the higher heating and cooling rates may be used.

Continuous annealing temperature: Ac₁ transformation point to (Ac₃ transformation point - 20°C)

With the continuous annealing temperature of less than the Ac₁ transformation point, the martensite phase is not formed after annealing, while with the continuous annealing temperature of over (Ac₃ transformation point - 20°C), the desirable aggregation structure formed in box annealing is lost due to transformation, thereby failing to obtain the produced sheet having a high r value. Therefore, the continuous annealing temperature is Ac₁ transformation point to (Ac₃ transformation point - 20°C). The retention time of continuous annealing is preferably as short as possible in order to ensure the production efficiency, the fine structure and the amount of dissolved N. From the viewpoint of stability of the operation, the retention time is preferably 10 seconds or more. Also, in order to ensure the fine structure and the amount of dissolved N, the retention time is preferably 120 seconds or less. From the viewpoint of stability of material properties, the retention time is preferably 20 seconds or more.

### Cooling after continuous annealing: cooling to the temperature region of 500°C or less at a cooling rate of 10 to 300°C/s

Cooling after soaking by continuous annealing is important for making fine the structure, forming the martensite phase, and ensuring the amount of dissolved N. In the present invention, cooling is continuously carried out to the temperature region of at least 500°C or less at a cooling rate of 10°C/s or more. With a cooling rate of less than 10°C/s, a necessary amount of martensite phase, a homogeneous fine structure and a sufficient amount of dissolved N cannot be obtained. On the other hand, with a cooling rate of over 300°C/s, homogeneity in material properties of the steel sheet in the width direction deteriorates due to a significant increase in the amount of supersaturated dissolved C. When the stop temperature of cooling at a cooling rate of 10 to 300°C/s after continuous annealing exceeds 500°C, refinement of the structure cannot be attained.

### Over aging condition: retention in the temperature region of 350°C to the cooling stop temperature for 20 seconds or more subsequent to cooling after continuous annealing

Over aging may be performed by retention in the temperature region of 350°C to the cooling stop temperature for 20 seconds or more subsequent to the stop of cooling after soaking by continuous annealing. By over aging, the amount of dissolved C can be selectively decreased, while the amount of dissolved N is maintained. With the retention temperature region of less than 350°C, a long time is required for decreasing the amount of dissolved C to cause a reduction in productivity. Therefore, the temperature region is preferably 350°C or more.

By retention in the temperature region of 350°C to the cooling stop temperature for 20 seconds or more, the amount of dissolved C can be decreased to achieve a higher degree of non-aging properties at room temperature. By increasing the retention time, further improvement can be expected, but the effect is saturated with the retention time of about 120 seconds. Therefore, the retention time is preferably 120 second or less.

In order to obtain a larger amount of strain age hardening, it is advantageous to use either of dissolved C and dissolved N. However, by using dissolved C, aging deterioration at room temperature becomes significant, thereby limiting parts to which the steel sheet is applied. Therefore, in order to produce a strain age hardenable steel sheet having versatility, over aging is preferably performed with the sufficient amount of dissolved N being ensured.

In producing a high-tensile-strength cold-rolled coated steel sheet comprising a high-tensile-strength cold-rolled steel sheet and a hot-dip coated layer formed on the surface thereof, continuous annealing after box annealing can be performed in a continuous hot-dip coating line comprising hot-dip galvanization subsequent to cooling after continuous annealing or further alloying to produce a hot-dip galvanized steel sheet.

### Temper rolling or lever processing: elongation of 0.2 to 15%

In the present invention, in order to correct the shape and control roughness, temper rolling or leveler processing may be carried out subsequent to the cold rolling step. When the total elongation of temper rolling or leveler processing is less than 0.2%, the desired purpose of correcting the shape and controlling roughness cannot be achieved. On the other hand, with a total elongation of over 15%, ductility significantly deteriorates. It is confirmed that the processing system of temper rolling is different from that of leveler processing, but the effects of both processes are substantially the same. Temper rolling and leveler processing are effective after plating.

For reference, description will now be made of forming conditions and conditions for subsequent heat treatment for increasing strength when the steel sheet of the present invention is molded, for example, press-molded. When the steel sheet of the present invention is subjected to press working, for example, deep drawing, the strain introduced by press working is several % to several tens%. Although the amount of strain changes with molded parts, a strain of about 5 to 10% is introduced into an inner plate and a structural member in the automobile field.

These automobile parts are heat-treated by coating and baking. However, with the steel sheet of the present invention, strength of a molded product can be effectively increased after heat treatment. In the present invention, as a method of evaluating burning hardenability in a laboratory, a tensile test specimen of JIS No. 5 size is obtained from the steel sheet in the rolling direction, and tensile strain of 10% is applied to the tensile test specimen by a tensile testing machine. Then, the specimen is heat-treated and again subjected to a tensile test. Particularly, when properties are evaluated after heat treatment in a low temperature region, the heat treatment conditions include 120°C and 20 minutes. In this test, the properties of the completed portion after heat treatment subsequent to press forming are evaluated.

Namely, in the present invention, the difference (ΔTS) between the tensile strength of the specimen after application of tensile strain and heat treatment and the tensile strength of a product is defined as the strength increasing ability of heat treatment.

In order to increase the strength of the molded product, the amount of strain introduced by forming, or the heat treatment temperature after processing is preferably as high as possible.

However, with the steel sheet of the present invention, when the amount of applied strain is about 5 to 10%, the strength can be sufficiently increased even by heat treatment at a temperature lower than conventional heat treatment, i.e., a temperature of 200°C or less, after forming. However, with a heat treatment temperature of less than 120°C, the strength cannot be sufficiently increased with the low train applied. On the other hand, with the heat treatment temperature of over 350°C after forming, softening proceeds. Therefore, the temperature of heat treatment after forming is preferably about 120 to 350°C.

The heating method is not limited, and hot gas heating, infrared furnace heating, hot-bath heating, direct current heating, induction heating, and the like can be used. Alternatively, only a portion where strength is desired to be increased is selectively heated.

### Examples

In the examples below, the amount of dissolved N, the microstructure, tensile properties, the r value, strain age hardenability, and aging property were examined. The examination methods were as follows:

### (1) Amount of dissolved N

The amount of dissolved N was determined by subtracting the amount of precipitated N from the total N amount of steel determined by chemical analysis. The amount of precipitated N was determined by an analysis method using a constant-potential electrolytic method.

### (2) Microstructure

A test specimen was obtained from each of cold-rolled annealed steel sheets, and the microstructure of a section (C section) perpendicular to the rolling direction was imaged with an optical microscope or a scanning electron microscope. Then, the fraction of the ferrite texture and the type and the structure fraction of a second phase were determined by an image analysis apparatus.

### (3) Crystal grain diameter

In the present invention, the value used as the average crystal grain diameter was a higher one of the value calculated from a photograph of a sectional structure by a quadrature method defined by ASTM, and the nominal value determined from a photograph of a sectional structure by an intercept method defined by ASTM (refer to, for example, Umemoto et al.: Heat Treatment, 24 (1984), p334).

### (4) Tensile properties

A test specimen of JIS No. 5 was obtained from each of cold-rolled annealed steel sheets in the rolling direction, and a tensile test was carried out with a strain rate of 3 x 10⁻³/s according to the regulations of JIS Z 2241 to determine yield stress YS, tensile strength TS, and elongation El.

### (5) Strain age hardenability

A test specimen of JIS No. 5 was obtained from each of cold-rolled annealed steel sheets in the rolling direction, and a tensile strain of 5% was applied as pre-deformation. Then, the specimen was subjected to heat treatment corresponding to coating and baking at 170°C for 20 minutes, and a tensile test with a strain rate of 3 x 10⁻³/s was performed to determine the tensile properties (yield stress TSBH, tensile strength TSBH). Then, BH amount = YSBH - YS5%, and ΔTS = TSBH - TS were calculated. YS5% represents deformation stress in 5% pre-deformation of the produced sheet, YSBH and TSBH represent yield stress and tensile strength, respectively, after pre-deformation and heat treatment, and TS represents the tensile strength of the produced sheet.

### (6) Measurement of r value

A test specimen of JIS No. 5 was obtained from each of the cold-rolled annealed steel sheets in each of the rolling direction (L direction), the direction (D direction) at 45° with the rolling direction, and the direction (C direction) at 90° with the rolling direction. The width-direction strain and thickness-direction strain of each of the test specimens were determined when a uniaxial tensile strain of 15% was applied to each specimen, and the r value of each specimen in each of the directions was determined from the following ratio of width-direction strain to thickness-direction strain: $r = ln ( w / w 0 ) / ln ( t / t 0 )$
(wherein w0 and t0 represent the width and thickness of a specimen before the test, and w and t represent the width and thickness of a specimen after the test).
The mean value was determined by the following equation: $r mean = ( r L + 2 r D + r D ) / 4$
wherein rL represents the r value in the rolling direction (L direction), rD represents the r value in the direction (D direction) at 45° with the rolling direction, and rL represents the r value in the direction (C direction) at 90° with the rolling direction. In order to improve the precision of experiment, calculation was made by using changes in elongation strain and strain in the width direction on the assumption that the volume was constant.

### (7) Aging properties

A test specimen of JIS No. 5 was obtained from each of cold-rolled annealed steel sheets in the rolling direction, and then subjected to aging at 50°C for 200 hours, followed by a tensile test. The difference in yield elongation ΔY-El between before and after aging was determined from the obtained results to evaluate aging properties at normal temperature. When ΔY-El was zero, it was evaluated that the specimen has non-aging properties and excellent natural aging resistance.

### (8) Tensile strength after forming and heat treatment

A test specimen of JIS No. 5 was obtained from each of produced sheets in the rolling direction, and then a pre-strain of 10% was applied thereto. Then, heat treatment was conducted for 20 minutes at a conventional heat treatment temperature of 120°C and a temperature of 170°C corresponding to coating and baking, and then tensile strength was determined.

### (9) Decrease (ΔEl) in total elongation by natural aging

The decrease (ΔEl) in total elongation by natural aging was determined as the difference between the total elongation measured with a specimen of JIS N0 5 obtained from the produced sheet in the rolling direction, and the total elongation measured with a specimen of JIS N0 5 separately obtained from the produced sheet in the rolling direction after accelerated aging (retention at 100°C for 8 hours) of natural aging.

### Example 1

Examples of the present invention are described below.

Melted steel having each of the compositions shown in Table 1 was formed in an ingot by a converter, and then formed in a slab by a continuous casting method. Each of the steel slabs was heated (in some cases, a hot slab was charged) and roughly rolled under the conditions shown in Table 2 to form a sheet bar. The sheet bar was then hot-rolled by the hot rolling step comprising finish rolling under the conditions shown in Table 2 to form a hot-rolled sheet. With some of the sheet bars, the adjacent sheet bars were bonded by the melt welding method, and then continuously rolled.

Each of the resultant hot-rolled sheets was cold-rolled in the cold rolling step comprising pickling and cold rolling under the conditions shown in Table 2 to form a cold-rolled sheet. Each of the thus-obtained cold-rolled sheet was box-annealed and then continuously annealed under the conditions shown in Table 2. Some of the cold-rolled sheets were temper-rolled after the cold-rolled sheet annealing step. Box annealing may not be carried out. In all cases, the annealing temperature of box annealing was the recrystallization temperature or more.

The thus-obtained cold-rolled annealed sheets were examined with respect to the amount of dissolved N, the microstructure, tensile properties, the r value, strain age hardenability, and the aging property.

The surfaces of the steel sheets of Nos. 17 and 18 were coated by hot-dip galvanization in an in-line after continuous annealing shown in Table 2 to form coated steel sheets. The coated steel sheets were also examined with respect to the same properties as described above.

The results are shown in Table 3.

All the examples of the present invention have excellent ductility, extremely high stable BH amount and ΔTS, excellent strain age hardenability, a mean r value of as high as 1.2, and natural non-aging properties. The properties of the hot-dip galvanized steel sheets of Nos. 17 and 18 shown in Table 3 are substantially the same as the cold-rolled steel sheets subjected to continuous annealing. On the other hand, in the comparative examples out of the range of the present invention, ductility deteriorates, the BH amount and TS are low, or aging deterioration significantly occurs. Therefore, the comparative examples do not have all the intended properties, and thus cannot be said as steel sheets having sufficient properties.

Steel sheet No. 11 contains C and N in amounts out of the range of the present invention, and has an amount of dissolved N and a martensite amount lower than the range of the present invention. Therefore, the BH amount and ΔTS are decreased, and ΔY-El is increased. Steel sheet No. 12 contains Al, N/Al and N out of the range of the present invention, and has an amount of dissolved N lower than the range of the present invention, and the average crystal grain diameter of ferrite higher than the range of the present invention. Therefore, the BH amount and ΔTS are decreased, and ΔY-El is increased.

In steel sheet No. 13, the slab heating temperature and finisher delivery temperature FDT are out of the range of the present invention, the amount of dissolved N and the amount of martensite are lower than the range of the present invention, and the average crystal grain diameter of ferrite is higher than the range of the present invention. Therefore, the r value, the BH amount and ΔTS are decreased. In steel sheet No. 14, the coiling temperature after hot rolling is out of the range of the present invention, the amount of dissolved N and the amount of martensite are lower than the range of the present invention, and the average crystal grain diameter of ferrite is higher than the range of the present invention. Therefore, the r value, the BH amount and ΔTS are decreased.

In steel sheet No. 15, the continuous annealing temperature is out of the range of the present invention, martensite is not formed, and the average crystal grain diameter of ferrite is higher than the range of the present invention. Therefore, the BH amount and ΔTS are decreased, and ΔY-El is increased. In steel sheet No. 16, box annealing is not performed to fail to develop the desirable aggregation structure, deteriorating the r value. Also, the average crystal grain diameter of ferrite, and the area ratio of martensite are out of the range of the present invention.

### Example 2

Steel having the composition shown in Table 4 was formed in a slab by the same method as Example 1, and then heated and roughly rolled under the conditions shown in Table 5 to form a sheet bar having a thickness of 30 mm. The sheet bar was hot-rolled by the hot rolling step comprising finish rolling under the conditions shown in Table 5 to form a hot-rolled sheet. With some of the sheet bars, the adjacent sheet bars on the finisher entrance side after rough rolling were bonded together by the melt welding method, and then continuously rolled. The temperatures of the ends of the sheet bar were controlled in the width direction and the length direction by using an induction heating-type sheet bar edge heater and a sheet bar heater.

The thus-obtained hot-rolled sheet was cold-rolled by the cold rolling step comprising pickling and cold rolling under the conditions' shown in Table 5 to form a cold-rolled sheet having a thickness of 1.6 mm. Then, the cold-rolled sheet was box-annealed and then continuously annealed by a continuous annealing furnace under the conditions shown in Table 5. In all cases, the annealing temperature of box annealing are the recrystallization temperature or more.

The thus-obtained cold-rolled annealed sheet was examined with respect to the amount of dissolved N, the microstructure, tensile properties, the r value, and strain age hardenability by the same methods as Example 1. The tensile property of each cold-rolled annealed sheet was measured at ten positions in each of the width direction and the long direction to examine variations in yield strength, tensile strength and elongation. The variation is shown by a difference between the maxim and minimum of all measurements, for example, δYS = (maximum of YS) - (minimum of YS). The results are shown in Table 6.

All the examples of the present invention have excellent strain age hardenability and a high r value, and exhibit extremely high stable BH amount, ΔTS and mean r value regardless of variations in production conditions. It was also recognized that in the examples of the present invention, by performing continuous rolling and controlling the temperature of the sheet bar in the long direction and the width direction, the thickness precision and the shape of the produced steel sheet are improved, and variations in material properties are decreased.

### Industrial Availability

According to the present invention, a cold rolled steel sheet can be obtained, in which TS is greatly increased by press forming and heat treatment while maintaining excellent deep drawability in press forming. The cold-rolled steel sheet has the excellent effect of industrially producing coated steel sheets by electro-galvanization, hot-dip galvanization, alloying hot-dip galvanization.

## Claims

1. A high-tensile-strength cold-rolled steel sheet having a high r value and excellent strain age hardenability and natural aging resistance comprising a composition, by mass %,
C: 0.025 to 0.15%;
Si: 1.0% or less;
Mn: 2.0% or less;
P: 0.08% or less;
S: 0.02% or less;
Al: 0.02% or less; and
N: 0.0050 to 0.0250%;
wherein N/Al is 0.30 or more, the amount of dissolved N is 0.0010% or more, the balance is composed of Fe and inevitable impurities, the structure is composed of a ferrite phase having an average crystal grain diameter of 10 µm or less at an area ratio of 80% or more and a martensite phase as a second phase at an area ratio of 2% or more, and the r value is 1.2 or more.

2. A high-tensile-strength cold-rolled steel sheet according to Claim 1, wherein the composition further comprises at least one of the following groups d to g:
Group d: at least one of Cu, Ni, Cr and Mo in a total of 1.0% or less;
Group e: at least one of Nb, Ti and V in a total of 0.1% or less;
Group f: 0.0030% or less of B; and
Group g: one or both of Ca and REM in a total of 0.0010 to 0.010%, in expense of Fe.

3. A method of producing a high-tensile-strength cold-rolled steel sheet having a r value of as high as 1.2 or more, and excellent strain age hardenability and natural aging resistance comprising:
the hot-rolling step of roughly rolling a steel slab by heating to a slab heating temperature of 1000°C or more to form a sheet bar, finish-rolling the sheet bar so that the finisher delivery temperature is 800°C or more, and coiling the finish-rolled sheet at a coiling temperature of 800°C or less to form a hot-rolled sheet;
the cold rolling step of pickling and cold-rolling the hot-rolled sheet to form a cold-rolled sheet; and
the cold-rolled sheet annealing step of box-annealing the cold-rolled sheet at an annealing temperature of the recrystallization temperature to 800°C, then continuously annealing the annealed sheet at an annealing temperature of Ac₁ transformation point to Ac₃ transformation point 20°C), and then cooling the sheet to the temperature region of 500°C or less at a cooling rate of 10 to 300°C/s;
wherein the steel slab has a composition, according to claim 1.

4. A method of producing a high-tensile-strength cold-rolled steel sheet according to Claim 3, further comprising performing over aging in a temperature region of 350°C to the cooling step temperature for a residence tine of 20 seconds or more subsequent to cooling after the continuous annealing.

5. A method of producing a high-tensile-strength cold-rolled steel sheet according to Claim 3 or 4, wherein the composition further comprises, by mass %, at least one of the following groups d to g:
Group d: at least one of Cu, Ni, Cr and Mo in a total of 1.0% or less;
Group e: at least one of Nb, Ti and V in a total of 0.1% or less;
Group f: 0.0030% or less of B; and
Group g: one or both of Ca and REM in a total of 0.0010 to 0.010%, in expense of Fe.

## Patentansprüche

1. Ein Hochfestes, kaltgewalztes Stahlblech mit einem hohen r-Wert und exzellenter Reckalterungseigenschaft und Alterungsbeständigkeit, umfassend eine Zusammensetzung, in Gew.-%:
C: 0,025 bis 0,15 %;
Si: 1,0 % oder weniger;
Mn: 2,0 % oder weniger;
P: 0,08 % oder weniger;
S: 0,02 % oder weniger;
Al: 0,02 % oder weniger; und
N: 0,0050 bis 0,0250 %;
wobei N/AI 0,30 oder mehr ist, die Menge an gelöstem N 0,0010 % oder mehr ist, der Rest aus Fe und unvermeidbaren Verunreinigungen besteht, das Gefüge aus einer Ferritphase mit einem durchschnittlichen Kristallkorndurchmesser von 10 µm oder weniger bei einem Flächenverhältnis von 80 % oder mehr und einer Martensitphase als eine zweite Phase bei einem Flächenverhältnis von 2 % oder mehr besteht und der r-Wert 1,2 oder mehr ist.

2. Ein Hochfestes, kaltgewalztes Stahlblech nach Anspruch 1, wobei die Zusammensetzung ferner wenigstens eine der folgenden Gruppen d bis g umfasst:
Gruppe d: wenigstens eine von Cu, Ni, Cr und Mo in einer Gesamtmenge von 1,0 % oder weniger;
Gruppe e: wenigstens eine von Nb, Ti und V in einer Gesamtmenge von 0,1 % oder weniger;
Gruppe f: 0,0030 % oder weniger an B; und
Gruppe g: eine oder beide von Ca und REM in einer Gesamtmenge von 0,0010 bis 0,010 %, anstelle von Fe.

3. Ein Verfahren zum Herstellen eines hochfesten, kaltgewalzten Stahlblechs mit einem r-Wert von 1,2 oder mehr und exzellenter Reckalterungseigenschaft und Alterungsbeständigkeit, umfassend:
den Warmwalzschritt zum Vorwalzen einer Stahlbramme durch Erwärmen auf eine Brammen-Erwärmungstemperatur von 1000°C oder mehr zum Formen eines Vorblechs, Endwalzen des Vorblechs, so dass die Endlieferungstemperatur 800°C oder mehr ist und Aufwickeln des endgewalzten Blechs bei einer Aufwickeltemperatur von 800°C oder weniger zum Formen eines warmgewalzten Blechs;
den Kaltwalzschritt zum Beizen und Kaltwalzen des warmgewalzten Blechs zum Formen eines kaltgewalzten Blechs; und
den Glühschritt des kaltgewalzten Blechs von Kistenglühen des kaltgewalzten Blechs bei einer Glühungstemperatur der Rekristallisationstemperatur bis 800°C, dann Durchlaufglühen des geglühten Blechs bei einer Glühungstemperatur von Ac₁-Umwandlungspunkt bis Ac₃-Umwandlungspunkt - 20°C und dann Abkühlen des Blechs auf den Temperaturbereich von 500°C oder weniger bei einer Abkühlrate von 10 bis 300°C/Sek.;
wobei die Stahlbramme eine Zusammensetzung nach Anspruch 1 hat.

4. Ein Verfahren zum Herstellen eines hochfesten, kaltgewalzten Stahlblechs nach Anspruch 3, bei dem anschließend zum Abkühlen nach dem Durchlaufglühen ferner Überaltern in einem Temperaturbereich von 350°C zu der Abkühlschritttemperatur für eine Haltezeit von 20 Sekunden oder mehr durchgeführt wird.

5. Ein Verfahren zum Herstellen eines hochfesten, kaltgewalzten Stahlblechs nach Anspruch 3 oder 4, wobei die Zusammensetzung ferner wenigstens eine der folgenden Gruppen d bis g, in Gew.-%, umfasst:
Gruppe d: wenigstens eine von Cu, Ni, Cr und Mo in einer Gesamtmenge von 1,0 % oder weniger;
Gruppe e: wenigstens eine von Nb, Ti und V in einer Gesamtmenge von 0,1 % oder weniger;
Gruppe f: 0,0030 % oder weniger an B; und
Gruppe g: eine oder beide von Ca und REM in einer Gesamtmenge von 0,0010 bis 0,010 %, anstelle von Fe.

## Revendications

1. Tôle d'acier laminée à froid ayant une résistance à la traction élevée, ayant une valeur r élevée et une excellente aptitude au vieillissement par contrainte, ainsi qu'une excellente résistance au vieillissement naturel comprenant une composition, en % en masse :
C : 0,025 à 0,15 % ;
Si : 1,0 % ou moins ;
Mn : 2,0 % ou moins ;
P : 0,08 % ou moins ;
S : 0,02 % ou moins ;
Al : 0,02 % ou moins ; et
N : 0,0050 à 0,0250 % ;
dans laquelle N/Al est égal à 0,30 ou plus, la quantité de N dissous est égale à 0,0010 % ou plus, le reste étant composé de Fe et des impuretés inévitables, la structure étant composée d'une phase de ferrite ayant un diamètre de grain cristallin moyen de 10 µm ou moins, pour un rapport de section de 80 % ou plus, et une phase de martensite, en tant que seconde phase, pour un rapport de section de 2 % ou plus, et la valeur r étant égale à 1,2 ou plus.

2. Tôle d'acier laminée à froid ayant une résistance à la traction élevée selon la revendication 1, dans laquelle la composition comprend, en outre, au moins l'un des groupes suivants d à g :
groupe d : au moins l'un de Cu, Ni, Cr et Mo en une quantité totale de 1,0 % ou moins ;
groupe e : au moins l'un de Nb, Ti et V en une quantité totale de 0,1 % ou moins ;
groupe f : 0,0030 % ou moins de B ; et
groupe g : l'un ou les deux de Ca et REM, en une quantité totale de 0,0010 à 0,010 %, aux dépens de Fe.

3. Procédé de fabrication d'une tôle d'acier laminée à froid ayant une résistance à la traction élevée, ayant une valeur r qui peut atteindre 1,2 ou plus et une excellente aptitude au vieillissement par contrainte, ainsi qu'une résistance excellente au vieillissement naturel comprenant :
l'étape de laminage à chaud consistant à laminer grossièrement une brame d'acier en la chauffant jusqu'à une température de chauffage de la brame de 1 000 °C ou plus, afin de former un larget, à exécuter un brunissage de finition du larget, de telle sorte que la température de délivrance du finisseur soit de 800 °C ou plus, et un bobinage de la tôle ayant subi le brunissage de finition à une température de bobinage de 800 °C ou moins, afin de former une tôle d'acier laminée à chaud ;
l'étape de laminage à froid consistant en un décapage et un laminage à froid de la tôle laminée à chaud pour former une tôle laminée à froid ; et
l'étape de recuit de la tôle laminée à froid consistant en un recuit en pot de la tôle laminée à froid à une température de recuit comprise entre la température de recristallisation et 800 °C, puis en effectuant un recuit en continu de la tôle ayant subi le recuit à une température de recuit comprise entre le point de transformation Ac₁ jusqu'au point de transformation Ac₃ - 20 °C), puis en refroidissant la tôle jusqu'à la région de températures de 500 °C ou moins, à une vitesse de refroidissement de 10 à 300 °C/s ;
dans lequel la brame d'acier a une composition suivant la revendication 1.

4. Procédé de fabrication d'une tôle d'acier laminée à froid ayant une excellente résistance à la traction selon la revendication 3, comprenant en outre l'exécution d'un survieillissement dans une région de températures allant de 350 °C jusqu'à la température de l'étape de refroidissement pour un temps de séjour de 20 secondes ou plus, à la suite du refroidissement après le recuit en continu.

5. Procédé de production d'une tôle d'acier laminée à froid ayant une résistance à la traction élevée selon la revendication 3 ou 4, dans lequel la composition comprend en outre, en % en masse, au moins l'un des groupes suivants d à g :
groupe d : au moins l'un de Cu, Ni, Cr et Mo, en une quantité totale de 1,0 % ou moins ;
groupe e : au moins l'un de Nb, Ti et V, en une quantité totale de 0,1 % ou moins ;
groupe f : 0,0030 % ou moins de B ; et
groupe g : l'un ou les deux de Ca et REM, en une quantité totale de 0,0010 à 0,010 %, aux dépens de Fe.
